# EUROPEAN PATENT SPECIFICATION

(11) **EP 1 111 194 B1**
(45) Date of publication and mention of the grant of the patent: **31.08.2011**
(21) Application number: 00310811.5
(22) Date of filing: 05.12.2000
(51) Int. Cl.: F01D 11/12, F04D 29/52

(54) **Composite abradable material**
Abreibbares Verbundmaterial
Matériau composite abradable

(30) Priority: 23.12.1999 US 471758
(43) Date of publication of application: 27.06.2001
(73) Proprietor: United Technologies Corporation, Hartford, CT 06101 (US)
(72) Inventor: Putnam, John W., Glastonbury, Connecticut 06033 (US); Watson, Charles R., Windsor, Connecticut 06095 (US)
(74) Representative: Leckey, David Herbert

(56) References cited:
- WO-A-98/35360
- US-A- 3 547 455
- US-A- 3 575 427
- US-A- 5 364 543
- US-A- 5 472 315

## Description

This invention relates to resilient composite abradable materials, and particularly to abradable materials for use in the compressor sections of gas turbine engines, and particularly in the low compressor section of such engines.

Modem large gas turbine engines have axial flow compressors which include multiple circular airfoil arrays mounted at the periphery of rotatable disks. Adjacent each set of moving compressor airfoils is an array of stationary airfoils. The efficiency of such a compressor is strongly affected by air which leaks around the ends of the moving airfoils. The typical approach to minimize such leakage is to provide an abradable air seal with which the compressor airfoil outer ends interact to minimize leakage.

U.S. patent 3,575,427 describes the abradable seal materials similar to those which are currently in use in engines produced by the present applicant. The seal material of U.S. patent 3,575,427 comprises a resilient matrix material containing a dispersion of friable hollow glass microspheres.

Applicants currently use such materials which comprise a silicone rubber matrix containing 15 to 50 volume percent of hollow glass microspheres as an abradable air seal material.

US 3,547,455 describes a further abradable seal, which uses hollow particles in an epoxy matrix. WO 98/35360 discloses a conductive composition comprising conductive filler particles in a resinous matrix.

The evolution of gas turbine engines has been in the direction of higher operating temperatures. Temperatures in the compressor section of the engine have increased moderately, while temperatures in the combustor in turbine section have increased substantially since the development of the material described in U.S. patent 3,575,427.

In gas turbine engines with glass microballoon containing seals, when the abradable seals abrade, the glass microspheres are carried through the combustor and turbine sections of the engine. In modern engines, the temperatures in the combustor and turbine sections, are sufficiently high to cause the glass microspheres to soften or melt. It has been occasionally observed that these softened or melted glass microspheres have adhered to engine components and have blocked air cooling holes. Blockage of cooling holes is detrimental to engine component longevity.

Accordingly, it is an object of this invention to describe an abradable material for use in modern high temperature gas turbine engines. It is another objective of the invention to describe an abradable material which whose constituents will not subsequently adhere to combustor and turbine components. It is yet another object of the invention to describe a compressor of abradable material which exhibits higher erosion resistance over temperatures ranging from room temperature to 204°C (400°F) than the currently used material and is usable in temperatures up to 232°C (450°F) and exhibits desirable abradability characteristics.

According to the invention there is provided an abradable material as claimed in claim 1.

In a preferred embodiment, the invention provides a high temperature resilient material comprising a high temperature capable silicone polymeric material which contains a dispersion of high temperature capable organic particles. The particles are preferably selected from a material which is stable to at least 204°C (400°F). The particles are preferably present in the seal in an amount of about 10 wt %.

The silicone polymeric matrix is selected so as to be thermally stable at temperatures in excess of 149°C (300°F) and preferably in excess of 232°C (450°F). Most preferably the silicone polymeric matrix can withstand short temperature spikes of up to 288°C (550° F) without undue deterioration.

This invention in various embodiments comprises a matrix containing a particle or low aspect ratio (<10:1) fiber dispersion.

The phrase "abradable silicone polymer matrix" or ASPM is used herein as a defined term for a material that is a resilient one or two part silicone polymer preferably catalyzed by a precious metal selected from the group consisting of Ru, Rh, Pd, Os, Ir, Pt and mixtures thereof, which is thermally stable at at least 149°C (300°F). The cured ASPM material preferably has a room temperature tensile strength of greater than 2.76 Nmm⁻² (400 PSI), an elongation to failure of greater than 100%, and a Shore A (Durometer) hardness of from 15-75, more preferably 15-50.

Preferably the ASPM material is a dimethyl or methyl phenyl silicone.

Preferably the ASPM material contains a transition metal oxide selected from the group consisting of oxides of V, Cr, Ce, Mn, Fe, Co, Ni, or other transition metal and mixtures thereof with iron oxide being particularly preferred. The transition metal oxide acts as a thermal or thermal oxidative stabilizer.

Preferably the ASPM material is produced from a mixture of a vinyl terminated polymer having a molecular weight of 1,000 g/mol to 1,000,000 g/mol; a silane crosslinker having a molecular weight of 300 g/mol to 10,000 g/mol and a precious metal catalyst, most preferably Pt. The ASPM may also contain a reinforcing file such as fumed silica.

Preferably the room temperature tensile strength of the cured ASPM material exceeds 6.9 Nmm⁻² (1,000 PSI).

Preferably the room temperature elongation to failure of the cured ASPM material exceeds 800%.

Preferably the Shore A Durometer hardness of the cured ASPM material is from about 15 to about 40.

Preferably the cured ASPM material is oxidation resistant, exhibiting less than 2% weight loss after 100 hours (using a 25.4 mm x 25.4 mm x 6.3 mm (1" x 1" x¼") sample) at 149°C (300°F), and most preferably at 204°C (400°F) exposure in air.

Preferably the cured ASPM material is thermally stable, losing less than 20% of its tensile strength after 100 hours a 149°C (300° F), and preferably 204°C (400°F).

The phrase "abradable organic filler particles" or AOFP is used herein as a defined term meaning a material that is hard, organic, and that retains useful properties at 149°C (300°F). The AOFP material must contain less than about 2% S to ensure proper curing of the ASPM material. The AOFP material must have a glass transition temperature which exceeds 300° F (149°C) and a room temperature impact strength in excess of 26,7J/m (0.5 ft-lb/in) to reduce the likelihood of particle breakage during abrading conditions in engine operation.

Preferably the AOFP material retains useful mechanical properties at temperatures in excess of 260°C (500°F).

Preferably the AOFP material contains less than about 2 wt% F so that the products of AOFP material combustion are not corrosive to gas turbine materials.

Preferably the AOFP material contains less than about 1 wt% S and less than about 1 wt% F.

Preferably the AOFP material produces only gaseous combustion products when combusted in a gas turbine engine at temperatures in excess of 1093°C (2,000°F) generally oxidizing conditions.

Many organic materials contain fillers such as mica, glass particles etc. Preferably the AOFP material does not contain fillers. If fillers are present they must either combust completely, or be non combustable with softening temperatures in excess of 1371°C (2500°F) and preferably in excess of 1649°C (3000°). Non combustable fillers preferably have a particle size of less than 0.025 mm (1 mil).

Preferably the AOFP material has a glass transition temperature exceeds about 204°C (400° F).

Preferably the AOFP material has a Deflection Temperature, measured according to ASTM D 648, at 1.8 MPa, which exceeds about 240°C (400°F), and preferably exceeds 260°C (500° F).

Preferably the AOFP material has a room temperature tensile strength which exceeds 68.9 Nmm⁻² (10 ksi).

Preferably the AOFP material has a room temperature elongation to failure which exceeds 1%.

Preferably the AOFP material has a room temperature Izod impact strength which exceeds 53,3 J/m (1,0 ft-lb/in).

The particles which are added to the matrix material serve to slightly weaken the matrix material, and make it more abradable. It is well within the ability of one skilled in the art to select the proper amount of particulate material for a matrix material having particular qualities to achieve the desired degree of abradability. We prefer to use from about 5 to about 20 weight percent particles.

The particles are selected from the group consisting of polyamides, polyimides, polyamide-imides.

We particularly prefer a polyamide-imide known as Torlon 4000 which is available from the BP Amoco Company of Chicago, Illinois. We prefer to use this material in an average particle size of 55 micrometers. A range of 35 to 75 micrometers appears to be a broad range for the average particle size. We prefer that 90% of particles have a size which is less than about 150 micrometers and that 90% of the particles fall in the size range of 10 to 125 micrometers.

Exemplary ASPM materials include:
a) LSR 5820 produced by the NuSil Company.
b) LSR 5830 produced by the NuSil Company.
c) Dow Corning Silastic GP-70 produced by the Dow Corning Company.
d) Visilox V-240 produced by the Rhodia Company.

Currently LSR 5830 is preferred.

Exemplary APM materials include:
a) Torlon available in several grades from BP-Amoco.
b) PMR-15, a NASA developed polyimide material commercially available from multiple sources, including Hycomp Corporation of Cleveland Ohio.
c) DMBZ, a NASA developed polyimide material commercially available from multiple sources including Hycomp Corporation

We currently prefer Torlon 4000 available from BP-Amoco.

In the gas turbine compressor application the seal material will generally be located on the radially interior surface of a ring, which is located in the engine so that it circumscribes the tips of the moving airfoils, and the abradable seal will preferably be located in a shallow groove or depression in the ring The depression will have a width which is comparable to and somewhat greater than the width of the compressor blades which will interact with the seal, for example 35-75 mm, and a depth of from 1 to 5 millimeters

The ring will be metallic, typically aluminum or titanium, and may be formed in segments. The seal material is applied to the groove in the ring or ring segment as follows. The groove is cleaned using conventional techniques. We prefer to anodize the cleaned groove surface when producing new parts, when overhauling parts, we have used chromate conversion coating such as Iridite 14-2 from the MacDermid Company in Wallingford, CT on the groove surfaces. Anodizing and chromate conversion are preferred but may not be required for all applications.

While the invention materials previously described will adhere to metallic surfaces, whether bare, anodized or with a chromate conversion coating, adherence is generally improved through the use of an appropriate primer material which is applied to the surface prior to the application of the particulate filled polymer material. The primer material will generally be supplied or specified by the silicone matrix supplier, typical generally useful primers include DC-1200 primer from Dow Coming Company of Midland MI, Visilox V-06 from the Rhodia Corporation of Troy NY and SP270 from the NuSil Corporation of Carpenteria, CA.

The ring or ring segment is provided with a mandrel which conforms to the inner surface of the ring sealing the groove and leaving an annular cavity to accept the particle filled silicone sealer of the invention. The mandrel has one or more apertures through which the silicone polymeric particle containing material can be injected.

The silicone polymeric particle containing material is injected into and fills the annular cavity. After the annular cavity is filled the apertures through which the material has been injected are closed and the filled ring or ring segment (along with the mandrel) is placed in an oven for curing. Curing is typically performed at temperatures between 149°C (300°F) and 204°C (400°F) for times of one to two hours or as otherwise recommended by the silicone producer.

After curing, the ring and mandrel are removed from the oven, the mandrel is removed, and the ring segment with the groove containing the silicone/particulate abradable rather may be further heat cured as appropriate.

The present invention will be better understood through reference to the following examples which are meant to be illustrative rather than limiting

LSR 5820 or LSR 5830 (produced by the NuSil Corporation; LSR 5820 and LSR 5830 have Shore A Durometer hardnesses of about 20 and 30 respectively after curing) which has been thermally modified with iron oxide is combined with 10 weight per cent of Torlon 4000TF particles having an average size of 55 µm, and the filled silicone material is processed and cured as previously described, 2 hours a 149°C (300°F) and 2 hours a 204°C (400°C). The system is available as R3-2160 from the NuSil Corporation. '

Typical properties for the cured R3-2160 are a Shore A hardness of 32, a tensile strength of 4.69 Nmm⁻² (680 psi) and a tensile elongation of 600%.

Seals fabricated from the resulting product provide equivalent abradability and 1.9 and 2.4 times the erosion life of current abradable seal materials (containing glass microballoons and as generally described in US 3,575,427) when tested at room temperature and 204°C (400°F), respectively, in a laboratory erosion apparatus using 50-70 mesh Ottawa sand at 244ms ⁻¹ (800 feet per second) and a 20° incidence angle.

Although this invention has been shown and described with respect to detailed embodiments thereof, it will be understood by those skilled in the art that various changes, omissions, and additions in form and detail thereof may be made without departing from the scope of the claimed invention. For example, the term particle as used herein also encompasses low aspect ratio (<10:1) fibre dispersions.

## Claims

1. An abradable material **characterized in that** it comprises from about 5 to about 20 weight percent of Abradable Organic Filler Particles (AOFP) in an Abradable Silicone Polymer Matrix (ASPM), wherein the AOFP material contains less than about 2 wt% S, and wherein the AOFP material is selected from the group comprising polyimides, polyamides, polyamide-imides, and mixtures thereof.

2. An abradable material as claimed in claim 1 wherein the AOFP material contains less than 1 wt% S.

3. An abradable material as claimed in claim 1 wherein the AOFP particles have an average size of 30-80 micrometers.

4. An abradable material as claimed in any preceding claim wherein the AOFP material has a room temperature Izod impact strength in excess of 53.3 J/m 1.0 ft-lb/in.

5. An abradable material as claimed in any preceding claim wherein the AOFP material has a glass transition temperature in excess of 149°C (300°C).

6. An abradable material as claimed in any preceding claim wherein the abradable silicone polymer matrix comprises a dimethyl silicone or a methyl phenyl silicone.

7. An abradable material as claimed in any preceding claim wherein the ASPM contains a stabilizing material consisting of one or more transition metal oxides.

8. An abradable material as claimed in any preceding claim wherein the cured ASPM has a room temperature tensile strength which exceeds 2.76 N/mm² 400 PSI.

9. An abradable material as claimed in any preceding claim wherein the cured ASPM has a room temperature elongation which exceeds 100%.

10. An abradable material as claimed in any preceding claim wherein the ASPM has a room temperature Shore A Durometer hardness of 15-75.

11. An abradable material as claimed in any preceding claim wherein the AOFP material contains less than 2% F.

12. An abradable material as claimed in any preceding claim wherein the AOFP material contains less than 1% S and less than 1% F.

13. An abradable material as claimed in any preceding claim for use in a gas turbine compressor.

14. A gas turbine abradable seal which comprises:
a) at least a segment of a ring, said ring being metallic.
b) a groove in the inward surface of said ring.
c) an abradable material located in said groove, said abradable material being as claimed in any preceding claim.

## Patentansprüche

1. Abreibbares Material, **dadurch gekennzeichnet, dass** es von etwa 5 bis etwa 20 Gew% abreibbarer organischer Füllstoffpartikel (AOFP) in einer abreibbaren Silikonpolymermatrix (ASPM) aufweist, wobei das AOFP-Material weniger als etwa 2 Gew% S enthält, und wobei das AOFP-Material ausgewählt ist aus der Gruppe, die Polyimide, Polyamide, Polyamid-Imide und Gemische davon aufweist.

2. Abreibbares Material wie in Anspruch 1 beansprucht, wobei das AOFP-Material weniger als 1 Gew% S enthält.

3. Abreibbares Material wie in Anspruch 1 beansprucht, wobei die AOFP-Partikel eine durchschnittliche Größe von 30 bis 80 Mikrometern haben.

4. Abreibbares Material wie in einem vorangehenden Anspruch beansprucht, wobei das AOFP-Material eine Izod-Schlagzähigkeit bei Raumtemperatur hat, die 53,3 J/m (1,0 ft-lb/in) überschreitet.

5. Abreibbares Material wie in einem vorangehenden Anspruch beansprucht, wobei das AOFP-Material eine Glasübergangstemperatur hat, die 149 °C (300 °F) überschreitet.

6. Abreibbares Material wie in einem vorangehenden Anspruch beansprucht, wobei die abreibbare Silikonpolymermatrix ein Dimethylsilikon oder ein Methylphenylsilikon aufweist.

7. Abreibbares Material wie in einem vorangehenden Anspruch beansprucht, wobei die ASPM ein stabilisierendes Material enthält, das aus einem oder mehreren Übergangsmetalloxiden besteht.

8. Abreibbares Material wie in einem vorangehenden Anspruch beansprucht, wobei die gehärtete ASPM eine Raumtemperatur-Zugfestigkeit hat, die 2,76 N/mm² (400 PSI) überschreitet.

9. Abreibbares Material wie in einem vorangehenden Anspruch beansprucht, wobei die gehärtete ASPM eine Raumtemperatur-Dehnung hat, die 100 Prozent überschreitet.

10. Abreibbares Material wie in einem vorangehenden Anspruch beansprucht, wobei die ASPM eine Shore. A-Durometerhärte bei Raumtemperatur von 15 bis 75 hat.

11. Abreibbares Material wie in einem vorangehenden Anspruch beansprucht, wobei das AOFP-Material weniger als 2 Prozent F enthält.

12. Abreibbares Material wie in einem vorangehenden Anspruch beansprucht, wobei das AOFP-Material weniger als 1 Prozent S und weniger als 1 Prozent F enthält.

13. Abreibbares Material wie in einem vorangehenden Anspruch beansprucht, zur Verwendung in einem Gasturbinenkompressor.

14. Abreibbare Gasturbinen-Dichtung, die aufweist:
a) mindestens ein Segment eines Rings, wobei der Ring metallisch ist.
b) eine Rille in der Innenoberfläche des Rings.
c) ein abreibbares Material, das sich in der Rille befindet, wobei das abreibbare Material so ist wie in einem vorangehenden Anspruch beansprucht.

## Revendications

1. Matériau abradable **caractérisé en ce qu'**il comprend environ 5 % à environ 20 % en poids de particules de charge organique abradable (PCOA) dans une matrice polymère de silicone abradable (MPSA), dans lequel le matériau PCOA contient moins d'environ 2 % en poids de soufre, et dans lequel le matériau PCOA est sélectionné dans le groupe comprenant des polyimides, des polyamides, des polyamide-imides, et des mélanges de ceux-ci.

2. Matériau abradable selon la revendication 1, dans lequel le matériau PCOA contient moins de 1 % en poids de soufre.

3. Matériau abradable selon la revendication 1, dans lequel les particules PCOA ont une taille moyenne de 30-80 micromètres.

4. Matériau abradable selon l'une quelconque des revendications précédentes, dans lequel le matériau PCOA a une valeur de résistance au choc Izod à la température ambiante supérieure à 53,3 J/m (1,0 pied-livre par pouce).

5. Matériau abradable selon l'une quelconque des revendications précédentes, dans lequel le matériau PCOA a une température de transition vitreuse supérieure à 149 °C (300 °F).

6. Matériau abradable selon l'une quelconque des revendications précédentes, dans lequel la matrice polymère de silicone abradable comprend une diméthylsilicone ou une méthylphénylsilicone.

7. Matériau abradable selon l'une quelconque des revendications précédente, dans lequel la MPSA contient un matériau stabilisateur consistant en un ou plusieurs oxydes de métaux de transition.

8. Matériau abradable selon l'une quelconque des revendications précédentes, dans lequel la MPSA durcie a une résistance à la traction à la température ambiante qui est supérieure à 2,76 N/mm² (400 livres par pouce carré).

9. Matériau abradable selon l'une quelconque des revendications précédentes, dans lequel la MPSA durcie a un allongement à la température ambiante qui est supérieur à 100 %.

10. Matériau abradable selon l'une quelconque des revendications précédentes, dans lequel la MPSA a une dureté au duromètre Shore A à la température ambiante de 15-75.

11. Matériau abradable selon l'une quelconque des revendications précédentes, dans lequel le matériau PCOA contient moins de 2 % de fluor.

12. Matériau abradable selon l'une quelconque des revendications précédentes, dans lequel le matériau PCOA contient moins de 1 % de soufre et moins de 1 % de fluor.

13. Matériau abradable selon l'une quelconque des revendications précédentes, destiné à une utilisation dans un compresseur de turbine à gaz.

14. Joint d'étanchéité abradable pour turbine à gaz, lequel comprend :
a) au moins un segment d'un anneau, ledit anneau étant métallique ;
b) une gorge dans la surface orientée vers l'intérieur dudit anneau ;
c) un matériau abradable situé dans ladite gorge, ledit matériau abradable étant tel que revendiqué dans l'une quelconque des revendications précédentes.
